

# UNITED STATES PATENT OFFICE.

FRANCIS C. WELCH, OF BEVERLY, MASSACHUSETTS.

## PROCESS OF IMPROVING THE QUALITY OF MASON'S HYDRATED LIME

1,410,087.

Specification of Letters Patent. Patented Mar. 21, 1922.

No Drawing.

Application filed November 8, 1921. Serial No. 513,633.

(FILED UNDER THE ACT OF MARCH 3, 1883, 22 STAT. L. 625.)

To all whom it may concern:

Be it known that I, FRANCIS C. WELCH, a citizen of the United States, residing at Beverly, in the State of Massachusetts, have invented new and useful Improvements in the Processes of Improving the Quality of Mason's Hydrated Lime, of which the following is a specification:

This application is filed under the act of 10 March 3, 1883, under the terms of which, the applicant agrees that the invention described herein, if patented, may be used by the Government or any of its officers or employees in prosecution of work for the Government, or by any other persons in the United States without the payment to him of any royalty thereon.

Mason's hydrated lime is completely defined by the specifications for same, issued 20 by the American Society for Testing Materials, No. C6—21T. In these specifications, the distinction between mason's and finishing hydrate is based solely upon the plasticity: for finishing hydrate, the plasticity figure must be greater than 200. Practically, the two kinds of hydrate are distinguished by the fact that mason's hydrate cannot be used for the finishing coat of plaster. It is so lacking in plasticity that the 30 plasterer cannot spread it on the wall.

The evidence indicates that both kinds of hydrate consists mainly of particles of colloidal size, the difference being that in the finishing hydrate, these particles may be 35 readily separated from each other, while in the mason's hydrate, they are aggregated together in groups. Each group of particles is apparently surrounded by an envelope of water, and the cohesion between the particles 40 in a group is so strong that the group cannot be broken up into its component particles, even by the most severe grinding.

I find that if mason's hydrate is ground either in the presence of or mixed with a 45 drying agent, the drying agent destroys the water envelopes surrounding the groups, and the grinding then breaks down the groups into individual particles. This results in an improvement of plasticity such 50 that a mason's hydrate, so treated, can be used as a finishing hydrate.

As drying agents, I have found effective the following materials, but it is obvious that any materials of similar nature will answer

the purpose; those which absorb the water 55 physically slate, shale, kaolin, diatomaceous earth, tripoli, fine sand, clay; those which absorb the water chemically, calcined gypsum, quicklime, magnesia, or the oxides of barium, iron, and phosphorus. 60

As this operation depends upon the breaking up of the water envelope surrounding the groups of particles in the mason's hydrated lime, and the water comprising these envelopes has a certain definite vapor pressure 65 depending upon its temperature, the desired results can also be obtained by increasing the temperature of the hydrate or by increasing the temperature or lowering the humidity of a current of air passed over the 70 hydrate.

By heating the hydrate or by increasing the temperature or lowering the humidity of a current of air passed over the hydrate, the vapor pressure of the envelope of water 75 around the particles of the hydrate is greater than the vapor pressure of the water in the air, causing the water envelope to evaporate.

The quantity of drying agent which may 80 be added depends somewhat upon economic conditions. I have achieved satisfactory results with as low as one per cent by weight of the hydrate. Equally good results can be obtained with larger additions of material, 85 according to the dehydrating power and amount of grinding up to the point where the added material seriously affects the setting properties of the lime.

The duration of grinding depends upon 90 the type of equipment used, the power and quantity of the dehydrating agent and the degree of plasticity required.

Specifically, I find that if to a mason's hydrate is added one per cent of its weight of 95 quicklime and the mixture ground in a ball mill for 2 hours, the resultant product will be sufficiently plastic to meet the requirements for finishing hydrate (see A. S. T. M. specification cited above). 100

I claim:

1. The process of increasing the plasticity of mason's hydrated lime, which comprises the grinding of the mason's hydrated lime in contact with a drying agent. 105

2. The process of increasing the plasticity of mason's hydrated lime, which comprises the grinding of the mason's hydrated lime,

- with an admixture of a material which can absorb water physically.
3. The process of increasing the plasticity of mason's hydrated lime, which comprises 5 the grinding of the mason's hydrated lime with an admixture of shale.
4. The process of increasing the plasticity of mason's hydrated lime, which comprises the grinding of the mason's hydrated lime with an admixture of a material which can 10 absorb water chemically.
5. The process of increasing the plasticity of mason's hydrated lime, which comprises the grinding of the mason's hydrated lime with an admixture of quick lime.
6. The process of increasing the plasticity 15 of mason's hydrated lime which comprises the grinding of the mason's hydrated lime in a current of warm, dry air.
7. The process of increasing the plasticity of mason's hydrated lime, which comprises 20 grinding in a current of air the mason's hydrated lime at a temperature whereby the water in the hydrate is partially evaporated.

FRANCIS C. WELCH.